

## UNITED STATES PATENT OFFICE.

WESLEY G. NICHOLS, OF CHICAGO HEIGHTS, ILLINOIS, ASSIGNOR TO AMERICAN MANGANESE STEEL COMPANY, OF CHICAGO, ILLINOIS, A CORPORATION OF MAINE.

## HEAT TREATMENT OF MANGANESE STEEL.

No Drawing.

Application filed February 26, 1923. Serial No. 621,461.

To all whom it may concern:

Be it known that I, WESLEY G. NICHOLS, a citizen of the United States, residing at Chicago Heights, in the county of Cook and 5 State of Illinois, have invented certain new and useful Improvements in the Heat Treatment of Manganese Steel, of which the following is a specification.

This invention relates to a method of heat 10 treating manganese steel castings, and has for its primary object to provide a method of procedure which will greatly increase the quantity of castings that can be treated in a given furnace within a given period of 15 time without injury to the castings.

In the heat treatment of manganese steel castings in gas, coal, or oil fired furnaces the practice has been to establish approximate equilibrium of temperature between 20 the castings and furnace at the time of charging the furnace, this being accomplished by either allowing the furnace to cool down to about the temperature of the castings, or holding the castings in the 25 molds where they are protected from atmospheric changes until the furnace is drawn and ready to be recharged, and then shaking the castings out of the molds at approximately the furnace temperature, breaking 30 the heads and gates from the castings, and charging the castings as quickly as practicable into the furnace, which proceeding involves considerably more labor than the 35 prices warrant, while the high temperatures of the castings which the workmen have to contend with prevent cleaning the castings of sand sufficiently to admit of proper treatment. It has never been considered practicable to charge cold castings into a hot furnace 40 because the flame or gases in furnaces of the types named have been too severe and too unevenly distributed. The light sections would take the heat long before the heavy sections did, attaining in many cases 45 a red heat or from 1200 to 1400° F. before the heavy sections reached as much as 700 to 800° F. This would cause excessive expansion of the light sections accompanied by a tendency to pull away from the heavy

sections, or to check, or otherwise render the 50 castings unserviceable.

I have found that by the procedure of the present invention and the use of an electric furnace of the resistance type, manganese steel castings may be charged into the furnace at atmospheric temperature even though the furnace has a temperature of from 1100 to 1400° F. or even higher, without any damage being done to the castings, thereby saving the time heretofore consumed in cooling down the furnace to what was supposed to be a safe temperature to receive the cold castings, and saving the expense of the proceeding incident to introducing the castings hot from the molds 60 already alluded to, and avoiding the disadvantage of introducing into the heating furnace castings insufficiently cleaned of sand. 65

In carrying out the invention, since time is unavoidably consumed in the original 70 heating of the furnace to working temperature after a shut-down, the general practice has been to insert the first charge of castings into the furnace while the latter is cold, and then developing the heat. This involves no 75 special problem since the furnace starts at approximately the temperature of the castings, or at atmospheric temperature. Immediately upon removal of this first load, a succeeding load is ready for introduction 80 into the furnace. At this time the temperature of the furnace will be about 1300° F. in consequence of some loss incident to the opening of the furnace and removal of the charge in which the heating has been completed. The new load is introduced into the furnace at this temperature of, say 1300° 85 F. and the furnace door is immediately closed, but the current which was interrupted at the end of the previous treatment 90 is left off for a period of fifteen to thirty minutes after the introduction of this second charge and the closing of the furnace. At the end of this last-named period the temperature of the furnace will be found 95 to have dropped, in consequence of absorption of heat by the castings, to from 1075 to 1125° F. Current is now supplied to the

- resistance elements of the furnace and heat is developed thereby, but at a rate which is not materially in excess of the power of the castings to absorb the heat, so that at the 5 end of the first hour of application of power the temperature will be found not to have increased owing to continued absorption of heat by the charge of castings; it may have decreased as much as from 15 to 35° F.
- 10 At the end of the second hour the temperature will still be substantially about that at which it stood when the current was applied, but after the second hour temperature will be observed to gradually increase until 15 it attains the upper critical point beyond which it should not be permitted to go in the treatment of manganese castings. Having attained the highest temperature, the current is regulated to hold the furnace at 20 such temperature for the requisite period of time to insure complete heat treatment, when the current will be shut off, the furnace opened, the finished charge removed, and a 25 third charge immediately introduced with a repetition of the cycle of conditions already enumerated. By proceeding in this manner, great economy in current consumption and time required for each heat treatment, and consequent increase of furnace capacity for 30 a given expenditure of current, result. Moreover, the life of the furnace lining as well as other parts of the furnace is prolonged by the elimination of repeated cooling and heating of the furnace.
- 35 The procedure above outlined and the results mentioned are not practicable with furnaces of the gas, coal, or oil-fired types because in such furnaces the heat source is generally located in one part of the furnace and 40 the heating medium is forced in under pressure of air, with the result that the wall opposite the heat source is at higher temperature than the wall adjacent thereto; moreover, the roof develops a higher temperature 45 than the bottom of the furnace, with the result that certain castings or parts of castings to be heated attain a very high temperature while other castings or parts are comparatively cool, which condition causes undue 50 strains in the pulling away of the light sections from the heavy sections. With the electric furnace, each and every part of the furnace is at the same temperature, and even after the current is turned on the heat is so 55 diffused throughout the furnace that there is no chance for any part to attain a higher temperature than the other parts, and it is impossible to overheat any particular part of the furnace. This is evidenced by the fact 60 that the furnace temperature at the end of two hours is found to be approximately the same as it was at the beginning of the operation. With this uniformity of furnace temperature, each portion of the castings absorb 65 heat uniformly.

By the procedure of the present invention it is possible to heat treat manganese steel castings of any size and variation of section with safety and without danger of spoiling the castings. It is not necessary to allow the 70 heat treating furnace to cool to the temperature of the castings before introducing the latter; castings at atmospheric temperature as well as castings having a very high degree of heat can be charged into the same furnace 75 without any injury to the cooler castings; and the furnace can have a relatively high temperature, even as high as 1600° F., at the time of charging the castings without endangering the latter. As a result of these 80 conditions, all castings can be treated in a given length of time and at a lower cost of power, large furnace equipment can be eliminated, and the quantity of castings scrapped on account of furnace cracks can be greatly reduced.

I claim:

1. The improvement in the art of heat treating manganese steel castings, which consists in introducing castings to be heat treated, while at low temperature, into a furnace standing at relatively high temperature but with the interruption of the heat source, permitting the temperature of the furnace to fall for a time while the castings absorb the heat, 90 and thereafter generating heat in the furnace and raising the temperature to that required for completing heat treatment.

2. The improvement in the art of heat treating manganese steel castings, which consists in introducing castings to be treated into a furnace standing at relatively high temperature but with interruption of heat source, maintaining this condition until the castings absorb a substantial quantity of heat 100 stored in the furnace, then resuming generation of heat in the furnace at a rate approximately commensurate with heat absorption of the castings, and slowly bringing the castings to the upper limit required to complete 105 their treatment.

3. The improved method of heat treating castings, which consists in introducing the castings to be treated into a furnace at the high temperature at which the furnace stands following withdrawal of a completed 115 charge of castings but with interruption of heat source, continuing the interruption of heat until the newly introduced castings have absorbed a substantial quantity of heat 120 stored in the furnace, then renewing the heat source and generating heat while the same is being additionally absorbed by the castings, and ultimately attaining and maintaining the upper limit of heat required to complete 125 the treatment.

4. The improved method of heat treating manganese steel castings, which consists in interrupting the heat source of an electric furnace, removing a completely heat treated 130

charge of castings from the furnace, immediately introducing a new charge of manganese steel castings into the furnace with the heat source still interrupted, continuing the interruption of heat source until the castings have absorbed a substantial quantity of heat from the furnace, then renewing the generation of heat at the source at a rate commen-

surate with the heat absorption of the castings until necessary temperature is attained <sup>10</sup> for completing the heat treatment, and maintaining the last-named temperature until the treatment is complete.

Signed at Chicago, Illinois, this 18th day of February, 1923.

WESLEY G. NICHOLS.